

Sept. 8, 1970

D. S. JACKSON

3,527,415

FLAKE METALLIC PIGMENT MILLING

Filed May 15, 1967

2 Sheets-Sheet 1



INVENTOR  
Donald Stanley JACKSON

*D. S. Jackson*  
ATTORNEY

Sept. 8, 1970

D. S. JACKSON

3,527,415

FLAKE METALLIC PIGMENT MILLING

Filed May 15, 1967

2 Sheets-Sheet 2

EXAMPLE III



FIG. 4

EXAMPLE IV



FIG. 6

EXAMPLE I



FIG. 3

EXAMPLE III



FIG. 5

INVENTOR

Donald Stanley JACKSON

ATTORNEY

ATTORNEY

## 1

3,527,415

## FLAKE METALLIC PIGMENT MILLING

Donald S. Jackson, Hudson Heights, Quebec, Canada, assignor, by mesne assignments, to International Bronze Powders Limited, Montreal, Quebec, Canada, a corporation of Canada

Filed May 15, 1967, Ser. No. 638,317

Int. Cl. B02c 17/00, 23/00; C09c 1/62

U.S. Cl. 241—24

4 Claims

## ABSTRACT OF THE DISCLOSURE

To produce classified flake metallic pigments, coarse particles of metal are comminuted continuously in an inert liquid and the comminuted product separated into at least three fractions, and at least the separated fraction containing the coarsest size particles and liquid recycled to the comminuting operation and the remaining fractions either processed to recover the flake metallic particles from the liquid or recycled. The particle size of the separated fractions below the coarsest is preferably below the range from 300 to 100 mesh. At least one of the fractions not recycled to the comminuting operation may be sub-classified into at least two fractions of different particle size distribution, from which flake metallic particles are recovered.

This invention relates to the production of well classified flake metallic pigments.

Metal powders or pastes serving as pigment for paint are generically referred to as "bronze powders" or "bronze paste" even though made from metals or alloys of metals which do not have or give what is specifically known as bronze appearance. The expressions "bronze powder" or "bronze paste" and the expression "bronze paint" as herein used are each employed in the broad generic sense as including any of the metallic powders, pastes or paints, even though the same is used and relied upon to give a golden, yellow, silvery or other metallic appearance to an article or surface coated thereby. The present invention is characterized by being economical of operation and capable of producing a more classified pigment than other known methods of manufacture. Other advantages will become apparent upon description of the process.

Bronze powders are manufactured either from alloys of copper such as brass, in cases where a golden or yellow tint is required or from aluminum, where the paint is to have a silvery cast. Such present powders as above mentioned are made by either stamping the metal in small hammer mills and subsequently polishing the product so obtained by rotating brushes, or other devices with the addition of a small quantity of suitable lubricant, or by milling in a grinding medium consisting of an inert liquid with subsequent separation of the liquid grinding medium to the extent desired depending on whether a paste or dry powder is required. Characteristic processes are disclosed in U.S. Pats. 1,930,684; 1,954,462; 1,832,868; 2,112,497; 1,498,318; 1,932,741; 2,136,445 and 2,002,891. Polishing of pastes produced by the wet comminution process may be accomplished by methods such as that described in U.S. Pat. 2,591,245. Or, if the liquid medium is completely separated, by methods such as those described for stamped powders. By any of the methods described, pastes or powders of two distinct types may be produced. By choice of milling and polishing lubricants either a lac or "leafing" type or a non-leafing type can be produced. The term "lac" or "leafing" refers to the property of the flake metal particles to orient themselves on the surface of a suitable vehicle to produce a mirror-like metallic finish. The scope of this invention is understood to encompass both of these types of products.

## 2

In all of the above described methods of manufacture, classification of the primarily produced comminuted flake product is commonly employed. The purpose of classification in these processes is to return to the comminution circuit coarse material produced at the same time so as to allow continuous operation of the comminution device. The pigment so produced tends, however, to induce an objectionable grey or blue cast when used as a pigment for many applications. This arises because the effect of classification as normally employed is to control the upper size limit with no effect on the distribution of particle sizes below the sieve cut-off point. This is especially true in the sub-sieve range of particle sizes. The quantity and size distribution of fines can be controlled within certain limits by increasing the rate of circulation of product and return of oversize around the milling classifying circuit. There are, however, practical limits to this approach as the classifying equipment will become overloaded or classifying equipment of extremely large capacity will be required.

Having regard to the foregoing, it is an object of this invention to provide for the manufacture of bronze powder or paste with a more controlled particle size distribution than can be manufactured by the conventional processes in a convenient manner.

It has generally been found that fine aluminum pigments which are capable of passing through a 325 or 400 mesh screen are quite grey in hue. Pigments produced according to the teaching of this invention have a controlled particle size distribution and are much more brilliant and metallic in lustre and exhibit superior color purity. Polychromatic paint films prepared according to conventional formulations, when pigmented with aluminum paste produced according to this invention, when compared to similar films pigmented with aluminum pigment produced by conventional processes, were superior in gloss, brilliance and color purity, and exhibited higher reflectance as measured on a Colormaster Tri-Stimulus Colorimeter.

These results satisfy the general requirement that has emerged for metallic pigments of a classified character for such applications as polychromatic finishes or the pigmentation of plastics. See "Special Effects" December 1961, Modern Plastics and "Evaluation and Description of Metallic Colors," Society of Plastics Engineers Journal, volume 21, No. 12, 1965.

According to the invention coarse particles of a metal of the kind used for pigments are subjected to a wet comminution operation in a grinding circuit in which the metallic particles are maintained within an inert liquid. Liquid bearing the comminuted particles is withdrawn from the comminuting operation and classified into at least three fractions being two oversize fractions of different particle sizes and an undersize fraction. The fraction containing the coarsest particles is returned to the grinding circuit. The fraction containing particles of an intermediate size is removed from the circuit. The fraction containing the finest particles is preferably isolated and the particles separated from the liquid as an end product. The particles from the fraction of intermediate size as well as those from the fraction of finest size are usable as pigments.

In accordance with the invention, a further separation may be effected in which at least one of the fractions not returned to the grinding operation is subjected to further classification. In this operation the fraction is separated by another type of classifying operation from that used for the primary classification for example, differential settling, so as to obtain two or more fractions of narrower particle size distribution than the original fraction.

The invention will be described in more detail by reference to the accompanying drawings illustrating preferred aspects of the invention and in which,

FIG. 1 is a diagrammatic representation of apparatus suitable for carrying out the invention;

FIG. 2 is a diagrammatic representation of a type of classifier used in sub-classification of the finest particle size fraction from the apparatus of FIG. 1;

FIG. 3 is a diagrammatic representation of characteristics of a prior art product produced when all of the oversize is returned to the mill and the undersize is the sole end product;

FIG. 4 is a diagrammatic representation of characteristics of the fine product produced when an intermediate oversize product is removed and not returned to the mill.

FIG. 5 represents characteristics of the product resulting from the further classification of the product of FIG. 4;

FIG. 6 represents the characteristics of a product obtained by further classification of the product of FIG. 4 operated in a somewhat different manner from that of the procedure resulting in the product of FIG. 3.

More specific reference will now be made to the drawings.

A multideck classifying screen of a vibrating type is shown at 15. The screen 15 is provided with respective screens 15a, 15b and 15c. Cut foil scrap or other suitable feed and lubricant is fed to a ball mill 16 through a feed line 17 from a suitable source of supply (not shown) together with a solvent make-up proceeding through line 19 from a filter press 21 which acted to remove the solvent makeup from an already milled and screened fraction. The ball milled material from the mill 16 passes through the line 23 to the multideck screen 15. Oversize material passes from the tops of the screens 15a and 15b to the lines 25 and 26 and thence into an oversize return line 27 back to the ball mill 22.

An intermediate size fraction passes from the screen 15c through the line 29 to the filter press 21, where liquid is removed and recycled in the line 19 or reclaimed in the line 31. Undersize material passes through the line 33 also to a filter press 35 which separates the solids from the liquid.

The undersize solid product separated from the liquid by the filter press 35 and the intermediate product from the filter press 21 represent end products which are each usable as pigments.

Should it be desirable to sub-classify the undersize material instead of being taken to the filter press 35 it is lead to a differential settler 37. This device separates the undersize fraction into two sub-fractions whose constitution can be adjusted depending on the flow rate.

The choice of the intermediate screen 15c cannot be specified exactly because it depends on the mechanical construction of the screen and the sieve, and the methods of vibrating. The choice of the intermediate screen has to be made on the basis of examining the particle size distribution of the intermediate fraction and of the finest particle size fraction. A guide line in selecting the screens of effective sizes is that an attempt must be to cut the milled product into fractions of as close the same weight as possible. Generally speaking the intermediate screen may range between 300 mesh and 100 mesh.

Typical procedures will now be exemplified for the further explanation of the invention, by reference to the following examples.

#### EXAMPLE I

A ball mill with dimensions 3 feet long by 3 feet diameter was charged with 2,200 lbs. of steel balls of mixed size from  $\frac{1}{4}$  inch diameter to  $\frac{1}{2}$  inch diameter. Under equilibrium operating conditions a slurry of Varsol and aluminum flake powder containing 23% solids was transported at the rate of 172 lbs./hr. to a multideck vibratory screening device (30 inch) fitted with screens of graduated fineness from 80 mesh on the top deck to 325 mesh on the bottom deck. The product was the minus 325 mesh portion and was produced at the rate of 6 lbs./hr. of metal

solids. All of the oversize was returned to the mill together with 6 lbs. of raw cut foil scrap to maintain the circulating metal content of the system constant. Quantities of Varsol and lubricant were added sufficient to maintain a material balance in the system. The product was largely freed from the Varsol diluent by means of a filter press. The Varsol so separated was used to make up the Varsol requirements of the system. The properties of the product so produced were given in Table I, as a basis of comparison of a prior art product with a product of the present invention.

#### EXAMPLE II

See FIG. 3 and FIG. 4.

15 A ball mill with dimensions 3 feet long by 3 feet diameter was charged with 2,200 lbs. of steel balls of mixed size from  $\frac{1}{4}$  inch to  $\frac{1}{2}$  inch diameter. Under equilibrium operating conditions a slurry of Varsol and aluminum containing 21 percent solids was transported at the rate of 189 lbs./hr. to a multideck vibratory screening device fitted with screens of graduated fineness from 80 mesh on the top deck to 325 mesh on the bottom deck. The equipment was identical to that described in Example I. The primary product was the minus 325 mesh portion and was produced at the rate of approximately 5.1 lbs./hr. of metal solids. A minus 250 mesh plus 325 mesh oversize portion was collected separately as a second product at the rate of approximately 0.8 lb./hr. and thereby diverted from the oversize returned to the mill. 20 The remaining oversize was returned to the mill together with 6 lbs. of raw cut foil scrap to maintain the circulating metal content of the mill. Quantities of Varsol and lubricant sufficient to maintain a material balance in the system were added. The products so produced were largely separated from the Varsol diluent by means of a filter press. The Varsol so separated was used to make up the Varsol requirements of the system. The properties of the minus 325 mesh product are given in Table I.

#### EXAMPLE III

35 The minus 325 mesh product of Example II after passing through the 325 mesh screen and before separation from the Varsol diluent was passed through a settling device similar to that revealed in Canadian Pat. 554,038 (see FIG. 5) at a rate sufficiently great to produce two fractions, a coarse underflow fraction and a finer overflow fraction. The flow rate through the settling device was controlled to split the original minus 325 mesh product into an overflow fraction containing 10 percent of the original pigment and an underflow fraction containing 90 percent of the original pigment. The properties of these fractions are given in Table I.

#### EXAMPLE IV

40 The minus 325 mesh product of Example II, after passing through the 325 mesh screen and before separation from the Varsol diluent, was passed through a settling device as described in Example III at a rate greater than that used in Example III which was sufficient to 45 produce an overflow fraction containing 50 percent of the original pigment and an underflow fraction containing 50 percent of the original pigment.

45 The data of Table I reveals particle size distribution data obtained by microscopic examination of the pigments produced. This data was produced by dispersing the pigments in a collodion film, counting 1000 particles and classifying these particles into various size categories. These counts were reduced to percentage distributions based on particle size. While one can see that there has been, in general, a redistribution of particle sizes between the pigment of Example I and Example II it is not very apparent that this should lead to the noted improvement in tri-stimulus reflectivity. It is perhaps more apparent if this data is recalculated to show the relative quantity of reflective surface available in each

particle size range. This can be done by multiplying the particle size count in each size range by a factor proportional to the square of the average particle size. This assumes that the reflective surface available from these flake pigments is proportional to the area of one surface only. The derived reflective surface functions for each pigment can be plotted to show a cumulative increase in reflective surface up to 100 percent for the whole pigment and a differential distribution of reflective surface derived as a function of particle size for the different size ranges. This latter data are shown in FIG. 6.

It is apparent from the data of FIG. 6 that real differences exist between the pigment produced according to Example I and that produced according to Example II. While both pigments can be classified as minus 325 mesh pigments, that of Example I derives its reflective characteristics from two size classifications of particles and that of Example II is mono disperse. The visual effect produced from pigment produced according to the teaching of Example II is much cleaner with less suggestion of fine particle background behind the coarser particles.

It is possible to improve the degree of classification when operating according to the teaching of Example I by increasing the rate of withdrawal of metal Varsol slurry from the mill or comminution device. By this means one can produce pigments intermediate in character between that produced according to the teaching of Example I and that produced according to the teaching of Example II. However, to accomplish this one is required to utilize excessively large classifying equipment in order to handle the flow of metal-Varsol slurry. It is much more convenient and economical to achieve the desired classification by withdrawing an intermediate oversize product containing metal flakes somewhat coarser than the desired product. By this means overmilling is avoided. In addition it has been found that the coarser fraction (minus 250 mesh plus 325 mesh) product has considerable utility as a pigment and is a desirable product.

TABLE I.—PARTICLE SIZE COUNT (EXPRESSED IN MICRONS)

|                                          | Below 5<br>(percent) | 5-10<br>(percent) | 10-15<br>(percent) | 15-20<br>(percent) | 10-20<br>(percent) | 20-30<br>(percent) | 30-40<br>(percent) | 40-50<br>(percent) | Colormaster tri-stimulus<br>reading |      |      |
|------------------------------------------|----------------------|-------------------|--------------------|--------------------|--------------------|--------------------|--------------------|--------------------|-------------------------------------|------|------|
|                                          |                      |                   |                    |                    |                    |                    |                    |                    | R                                   | G    | B    |
| Example I (prior art).....               | 60.8                 | 19.6              | -----              | -----              | 14.7               | 1.9                | 2.4                | 0.5                | 35.9                                | 35.8 | 36.3 |
| Example II.....                          | 54.2                 | 26.4              | -----              | -----              | 14.7               | 3.3                | 0.9                | 0.4                | 36.8                                | 36.6 | 37.1 |
| Example III—10% overflow, 90% underflow: |                      |                   |                    |                    |                    |                    |                    |                    |                                     |      |      |
| Underflow (coarse).....                  | 55.5                 | 23.5              | -----              | -----              | 15.6               | 3.6                | 1.2                | 0.5                | 37.1                                | 37.0 | 37.4 |
| Overflow (fine).....                     | 84.5                 | 12.7              | 2.5                | 0.2                | -----              | -----              | -----              | -----              | 32.3                                | 32.0 | 32.6 |
| Example IV—50% overflow, 50% underflow:  |                      |                   |                    |                    |                    |                    |                    |                    |                                     |      |      |
| Underflow (coarse).....                  | 58.2                 | 20.7              | -----              | -----              | 15.0               | 4.3                | 1.2                | 0.6                | 37.8                                | 37.5 | 38.0 |
| Overflow (fine).....                     | 77.2                 | 14.6              | -----              | -----              | 6.8                | 1.2                | 0.2                | -----              | 34.2                                | 33.9 | 34.5 |

It is apparent from the results shown in Table I and FIGS. 5 and 6 that a further desirable classification of product in the sub-sieve range (minus 325 mesh) is achieved according to the teaching of Example III and Example IV. Depending on the extent which the minus 325 product of Example II is split into overflow and underflow fractions, the degree of classification of the superfine pigment (overflow fraction) can be controlled. By these two processes a logically related and well differentiated (in terms of particle size) series of pigments can be produced. The visual optical effects produced by these various pigments seem to depend not on the location of the peak in the curves shown in FIG. 6, but on the relative quantity of reflective surface at the coarse and fine end. Panels prepared using the two pigments produced by the method of Example IV are very different. The overflow pigment appears very much finer than the underflow pigment. The teaching of Examples III and IV constitute an extremely efficient method of producing classified pigments whose maximum particle size is much less than the effective control aperture of commercially

available screens. However, the same technique can be used if desired to differentiate the minus 250 mesh plus 325 mesh fraction into two derivative fractions.

It is not necessary to utilize a screening or sieving classification to achieve the purposes of this invention. It is obvious to anyone skilled in the art of classification that any type of classifier capable of producing at least three well defined products (in terms of particle size) from the primary mill output would be satisfactory. See for example Wilfley table and similar devices described in "Handbook of Mineral Dressing" Taggart, Wiley & Sons, 1945, Sections 11-62 to 11-90. Other types of classifiers may be used providing they meet the requirement of producing sufficient differentiation of particles based on flake diameter and sufficient fractions thereof. Similarly the scope of this invention is not limited to the use of ball mills. Any comminution device capable of applying impact pressure and frictional rubbing contact sufficient to break up and flatten out the metal particles and os completely to change their form into flake-like particles, will suffice for the practice of this invention. Similarly this invention is not restricted to the use of an overflow classifier of the type cited for secondary classification of the sub-sieve product. Any type of classifier capable of differentiation of the solvent borne flake particles in what is commonly known as the sub-sieve range of particle sizes into two or more fractions will suffice, e.g. liquid cyclone. Some such devices are cited in "Handbook of Mineral Dressing," Taggart, Wiley & Sons, 1945, Sections 8, 10 and 11.

The practice of this invention leads to a logically related series of flake metal pigments which vary in particle size from a size capable of being differentiated by a simple screening system to products in the sub-sieve range. All of these products are classified in that they have a desirable particle size distribution and as such especially valuable for pigmentation. The relationship of the pigments to the mode of producing them is shown in FIGS. 3, 4, 5 and 6.

I claim:

1. A method for manufacturing metallic flaked powders, comprising, continuously passing an inert liquid containing coarse particles of metal through a grinding circuit whereby they are comminuted, continuously withdrawing from the grinding circuit liquid containing the thus comminuted particles, classifying the withdrawn comminuted material into two oversize fractions of different particle sizes and an undersize fraction which is the desired classified product, and continuously returning to the grinding circuit only the coarsest of the two oversize fractions.

2. A method, as defined in claim 1, in which the finer of the oversize fractions removed from the grinding circuit has a particle size within the range from 300 to 100 mesh.

3. A method, as described in claim 1, in which the metal is aluminum.

4. A method, as defined in claim 1, in which the metal is a copper alloy.

References Cited  
UNITED STATES PATENTS

|           |         |         |          |
|-----------|---------|---------|----------|
| 1,930,684 | 10/1933 | Kramer  | 241—3    |
| 1,954,462 | 4/1934  | Tainton | 241—3    |
| 2,002,891 | 5/1935  | Hall    | 241—3 X  |
| 2,136,445 | 11/1938 | Kramer  | 241—30 X |
| 2,149,220 | 2/1939  | Krebs   | 241—20   |

|           |         |           |          |
|-----------|---------|-----------|----------|
| 2,272,629 | 2/1942  | Arthur    | 241—3    |
| 2,274,766 | 3/1942  | Ziehl     | 241—3    |
| 2,526,519 | 10/1950 | Jorgensen | 241—20   |
| 2,571,866 | 10/1951 | Greene    | 241—20 X |

5 LESTER M. SWINGLE, Primary Examiner  
D. G. KELLY, Assistant Examiner